

## UNITED STATES PATENT OFFICE

GEORGE A. RICHTER AND MILTON O. SCHUR, OF BERLIN, NEW HAMPSHIRE, ASSIGNEES  
TO BROWN COMPANY, OF BERLIN, NEW HAMPSHIRE, A CORPORATION OF MAINE

## PROCESS OF CHEMICALLY TREATING AND BLEACHING CELLULOSE PULP

No Drawing. Original application filed June 6, 1928, Serial No. 283,452. Divided and this application filed August 16, 1929. Serial No. 386,487.

This invention relates to the production of a bleached cellulose pulp of high cleanliness, whiteness, and low copper number.

In our Patent No. 1,639,704, dated August 23, 1927, it is disclosed that when free alkali is present during the bleaching of cellulose pulp, a product of high whiteness may be obtained without injury to the strength of the fibers and without lowering the alpha cellulose content of the pulp through the formation of oxycelluloses. The free alkali is preferably added to the bleach liquor at the start of bleaching and somewhat in excess of the amount necessary to be gradually consumed by reaction with acidic constituents initially present in the unbleached pulp or formed during bleaching, so that a distinctly alkaline condition is maintained throughout the bleaching operation. The alkali apparently makes the reaction between the bleach and pulp more selective in so far as the removal of impurities from the pulp is concerned. It also appears to have a solvent effect upon such oxycelluloses as may be present in the pulp at the start of bleaching, or as may be formed during bleaching. This patent further teaches the fact that higher temperature may be safely used during bleaching if free alkali be present in the bleach liquor, thereby eliminating the necessity for refrigerating the bleach liquor in hot weather, especially when stock is being bleached at a high density. Because of the protective influence which the alkali exercises over the cellulose, danger of local overbleaching is avoided, so that raw stock and strong bleach liquor may be uniformly admixed even in the summer when local overbleaching would ordinarily be certain to occur, particularly during initial mixing of the comparatively high temperature stock, resulting in a weakened stock and in a comparatively high bleach usage. A further advantage resulting from the use of free alkali during bleaching is the reduction in the number of resinous specks usually associated with the fibers, and accordingly the production of a cleaner pulp.

We have now found that if an alkali such as caustic soda is added to the raw stock before the bleach liquor, and is allowed to re-

main in contact therewith at about room temperature for several hours, it has better opportunity thoroughly to penetrate the stock and to loosen resinous specks. This initial treatment with alkali, while advantageous when using any type of bleach, is of marked advantage when calcium base bleach, such as calcium hypochlorite, is subsequently employed, for when the alkali and calcium hypochlorite are added simultaneously to the raw pulp, there is a tendency for the bleach to react with the resins to form insoluble resinate and oxidation products which become fixed on the pulp, thereby interfering to an appreciable extent with the solution or dispersion of the resins, and the attainment of high whiteness. Even when sodium hypochlorite bleach is subsequently used, the initial treatment with an alkali such as caustic soda is advantageous, in that the resins are peptized and brought into a condition more susceptible to attack and removal by the bleach. In our application Serial No. 283,452, filed June 6, 1928, various examples of initially treating the stock with alkali and then bleaching were given, one of these examples involving the addition of bleach to the alkaline liquor after the stock has been in contact with such alkaline liquor for a while. This application is a divisional of our application Serial No. 283,452, and is intended to cover such a procedure, which is especially advantageous in a mill where a continuous process is being practised, that is, where the pulp is caused to flow as a continuous stream of pulp suspension through a suitable system or apparatus. In such case, about  $\frac{3}{4}$  % caustic soda may be added to the raw stock, e. g., sulphite pulp, entering the system at 12% consistency and at about 70° F. At a point in the system reached by the stream pulp about two hours later, about 12% to 15% bleach may be added and the temperature raised to 80° F. About  $\frac{1}{2}$  % of the caustic initially added will be consumed in the two-hour treatment before the bleach is added, but the stock will remain in a distinctly alkaline condition until practically all the bleach is consumed.

In addition to the advantages hereinbefore

enumerated resulting from the application of the process of our invention, we have found that in actual mill practice we produce a final product of higher pH value than that associated with pulp bleached in the usual way. Thus, the raw stock bleached in the usual way resulted in a dry sheet of pulp, usually termed "dryer sheet" in the trade, having a pH value of about 3.2 to 3.6 when tested by staining with bromo-cresol green, but when processed as herein described, resulted in a dry sheet of pulp having a pH value of about 4.8 to 5.5. The higher pH value connotes greater stability in the pulp. Results obtained from large scale tests have shown that the stock of higher pH value will better endure a long-continued beating. When beaten, for example, together with rag stock, as is done in mills of limited beater capacity, the wood pulp fibers still have good strength when the tough rag fibers have been properly hydrated.

The process of the present invention has especial utility when applied in the treatment of raw sulphite pulp to produce a product which may be hydrated or gelatinized as readily as the usual sulphite pulp which has not been subjected to the process of this invention and is as suitable for the manufacture of hard, ratty papers of good strength and tear resistance, but of superior whiteness and cleanliness. The initial treatment of the raw pulp with weak solutions of alkali at about room temperature, as herein described, does not change the character of the fiber as to its alpha cellulose or pentosan content to a pronounced degree, but is more especially effective in the removal, or in facilitating the subsequent removal by bleaching, of troublesome bleach-resisting and coloring impurities which otherwise require a more drastic bleaching treatment and cause a product of inferior whiteness, cleanliness, and copper number, to result. Our process is practicable, in that it may be carried out with a low alkali and bleach consumption, without the use of heat in the preliminary step, and without requiring equipment other than that usually employed in a bleaching process.

While in the specific example given the alkalinity of the dilute solution at about room temperature used in the treatment of the pulp and in maintaining the bleach liquor alkaline is afforded by caustic soda, other chemicals, such as sodium carbonate, sodium phosphate, or borax may be used for this purpose. Again, while the specific example deals with the use of sulphite pulp as a raw material, and a process comprising essentially only the chemical treatment of bleaching after the initial alkali treatment, other pulps may be used as a raw material and other chemical treatments may be advantageously included. For instance, the treatment of pulp with a dilute caustic soda solu-

tion at about room temperature, followed by the addition of bleach to the solution, may be advantageously included as the final steps in a pulp refining process which comprises the step of digesting raw wood pulp at elevated temperature or at room temperature in an alkaline liquor of sufficient alkalinity to refine the pulp to high alpha cellulose content, or in a pulp refining process which comprises the step of treating the raw wood pulp with chlorine water or with bleach liquor before digesting in the alkaline refining liquor.

What we claim is:

1. A process which comprises treating cellulose pulp with a dilute alkaline solution at about room temperature, maintaining the pulp in contact with the solution for a substantial period of time, and adding bleach to the alkaline solution to whiten the pulp. 80
2. A process which comprises treating raw cellulose pulp with a dilute alkaline solution at about room temperature, and after a substantial amount of alkali has been consumed, adding bleach to the alkaline solution to whiten the pulp. 90
3. A process which comprises treating raw cellulose pulp with dilute caustic soda solution at about room temperature, and then, after awhile adding bleach to the solution in amount sufficient to whiten the pulp while the solution still contains sufficient caustic soda to maintain a distinctly alkaline condition throughout the bleaching operation. 95
4. A process which comprises treating a flowable aqueous suspension of raw sulphite pulp at about room temperature with about 3/4% caustic soda, based on the air-dry weight of pulp, and after a substantial amount of the caustic soda has been consumed, adding bleach to the pulp suspension. 100
5. A process which comprises treating a flowable aqueous suspension of raw sulphite pulp at about room temperature with about 3/4% caustic soda, based on the air-dry weight of pulp, and after about two hours' treatment, adding bleach to the pulp suspension to whiten the pulp. 110
6. In a process which involves the flow of unbleached pulp as a continuous stream of pulp suspension through a suitable system, those steps which comprise adding caustic soda to the stream to produce a dilute solution at about room temperature, and adding bleach at point in the system, reached by the stream considerably later but while it still contains sufficient caustic soda to maintain the pulp in a distinctly alkaline condition until practically all the bleach is consumed. 115

In testimony whereof we have affixed our signatures.

GEORGE A. RICHTER.  
MILTON O. SCHUR.